

E. S. LEAVER.  
APPARATUS FOR EXTRACTING METALS FROM THEIR ORES.  
APPLICATION FILED JULY 2, 1918.

1,312,488.

Patented Aug. 5, 1919.

2 SHEETS—SHEET 1.



*INVENTOR*

Edmund S. Leavens

E. S. LEAVER.

APPARATUS FOR EXTRACTING METALS FROM THEIR ORES.

APPLICATION FILED JULY 2, 1918.

1,312,488.

Patented Aug. 5, 1919.

2 SHEETS—SHEET 2.



INVENTOR

*Edward S. Leaver*

# UNITED STATES PATENT OFFICE.

EDMUND S. LEAVER, OF TUCSON, ARIZONA, ASSIGNOR OF ONE-HALF TO CHARLES E. VAN BARNEVELD, OF TUCSON, ARIZONA.

## APPARATUS FOR EXTRACTING METALS FROM THEIR ORES.

1,312,488.

Specification of Letters Patent.

Patented Aug. 5, 1919.

Application filed July 2, 1918. Serial No. 243,015.

*To all whom it may concern:*

Be it known that I, EDMUND S. LEAVER, a citizen of the United States, residing at Tucson, in the county of Pima, State of Arizona, have invented a new and useful Apparatus for Extracting Metals from Their Ores, of which the following is a specification.

This invention relates to an apparatus for extracting metals from their ores, using sulfurous acid as a leaching agent. The apparatus is adapted for extraction of copper, manganese and other metals.

The main object of the invention is to provide an apparatus which is adapted to extract the copper or other metal from the ore by the action of sulfurous acid and to oxidize the resulting compound so as to produce the sulfate of the extracted metal, such sulfate being adapted for further treatment to recover the metal therefrom. A further object of the invention is to provide an apparatus for the above stated purpose in which provision is made for maintaining proper conditions of temperature in each portion of the apparatus according to the action desired therein, so that the heat of the sulfurous gases coming from a sulfur burner or sulfid roasting apparatus and containing sulfur dioxid together with oxygen is utilized in heating the ore pulp so as to drive off the remaining sulfur dioxid therefrom and to cause oxidation of the sulfites in the solution, while the ore pulp supplied by the apparatus is being continually brought in contact with sulfurous gases cooled by the above described operation in the manner suitable for the most effective absorption of the gas and leaching of the ore.

The accompanying drawings illustrate an embodiment of my invention, and referring thereto:

Figure 1 is a side elevation of the apparatus.

Fig. 2 is a transverse section of the extracting and oxidizing drum taken on line 2-2 in Fig. 1.

Fig. 3 is a transverse section of said drum taken on line 3-3 in Fig. 1.

Fig. 4 is a section on line 4-4 in Fig. 1.

Fig. 5 is a partial longitudinal section of the drum on line 5-5 in Fig. 2.

My improved apparatus for ore extraction comprises a drum 1 mounted to rotate on

bearing rollers 2, or otherwise, and provided with means such as chute 3, for feeding ore pulp through an opening 5 at one end thereof, means such as outlet pipe 8 and launder 4 for discharging and carrying away ore pulp from the other end of the drum and means for forcing gas carrying sulfur, dioxid and oxygen through said drum in reverse direction or counter current to the movement of the ore pulp therein. I have indicated for this purpose a sulfur burner 6, of usual type connected to a blower or pump 7, by which the gases from said sulfur burner are forced through pulp outlet and gas inlet pipe 8 leading through opening 9' in a head 9 at one end of the drum 1. It will be understood, however, that in case sulfurous gases are available as a waste product, for example, gases from roasters in which sulfid ores are subjected to usual roasting operations—such gases may be utilized in my apparatus being forced directly by the pump 7 into the drum through the gas inlet 8. Said gas inlet also acts as a pulp outlet having a downwardly extending branch 10 which extends into the pulp discharge launder 4 and is provided with an opening 11 at its lowest portion through which the ore pulp flows into said launder.

The drum 1 may be of any suitable material resistant to the acid solution—for example, it may be made of wooden staves fastened together with bands or hoops 22 in the usual manner of cylindrical barrels 90 of this character and provided with wooden ends 9 and 14 having respectively central openings 9' and 5 for receiving respectively the pulp outlet pipe 8 and the pulp inlet pipe or chute 3. Packing means indicated 95 at 12 is preferably provided at opening 9' around gas inlet and pulp outlet pipe 8, to make a gas tight joint while permitting rotation of the drum. Said drum is provided with rings 15 surrounding the same 100 and secured thereto and running on the rollers 2 to rotatively support the drum, suitable means such as gearing 16 being connected to said rollers to rotate the drum.

The interior of the drum 1 is divided longitudinally by a series of transverse partitions 17, each of which is provided with a plurality of annular series of openings 19 and 20 through which the pulp may pass along the drum between successive sections 110

or spaces 21 which are separated by said partitions. The openings 20 in said partitions which are in the annular series nearer the peripheral wall 23 of the drum, are sufficiently large to receive longitudinal baffle rods or bars formed, for example as wooden strips 24 extending nearly the full length of the drum and through all of the transverse partitions 17, said baffle bars or strips extending through the holes or openings 20 and secured therein in any suitable manner. Said bars, however, do not completely fill said openings 20, but leave an open space 20' adjacent to each bar through which the pulp 5 may flow from section to section as aforesaid. These bars 24, do not extend into the last section 27 between the last partition 17 and the head 9 of the drum, and an open space 28 is also left between the other head 15 14 of the drum and the first partition. The last section 27 of the drum constitutes an elevating and discharging section, suitable elevating devices 30 consisting of radial wooden strips being secured in said section 20 and extending from the peripheral wall at 25 the drum inwardly to points intermediate the said peripheral wall and the axis of the drum. The pulp discharge pipe which also constitutes the gas inlet pipe, is located at the axis of the drum and has an open topped portion 8' extending into section 27 so that material elevated by the elevating devices 30 falls into said pulp discharging means 8 and is conducted thereby to the launder 4.

30 Drum 1 is also provided, throughout the sections 21, with bucket lifts 13, formed as ribs or flanges extending longitudinally of the drum and projecting from the wall of the drum inwardly and forwardly with respect to the direction of rotation of the drum.

35 The baffle bars 24 are arranged in a plurality of annular series, the bars in adjacent series being in staggered relations so that the material raised and then dropped by lifts 13 will be intercepted by said baffles and will descend from one baffle to another and will be thereby splashed and distributed so as to produce extended contact with the gases 40 in the drum.

45 The drum is operated by suitable driving means, such as gearing 16, so as to rotate the drum in the direction shown by the arrow in Fig. 2; the ore pulp being fed in through the chute, 3, and passing from the receiving to the delivery end of the drum by gradually finding its way through the openings 19 and 20, in the transverse partitions 17, so as to pass through all of the sections 21 successively.

50 In the rotation of the drum the bucket lifts 13, in their ascending movement, raise the ore pulp and as they reach the upper part of the drum drop the pulp onto the baffle bars or strips, 24, in such manner that

the ore pulp is splashed and distributed over the surfaces of the bars and on the transverse partitions and throughout the body of gas, in the form of descending drops or particles, so as to produce extended and intimate contact between the ore pulp and the sulfurous and oxidizing gases passing through the drum in counter current with the ore pulp. When the ore pulp reaches the final section, 27, the lifts, 30, in their revolving movement, 55 raise the pulp and drop it into the discharge or exit pipe, 8, whereby it is conducted through trap opening, 11, into launder 4.

55 The drum is operated so as to rotate at a speed of 15 to 20 revolutions per minute. 60 Pulp of the proper consistency (varying from 0.6 parts to 5 parts of water to 1 part of ore) fed into the drum at one end is met by a counter current flow of heated air carrying a varying percentage ( $\frac{1}{2}$  to 6%) of 65  $\text{SO}_2$  gas, which is forced into the drum through the gas inlet or pulp exit 8 under a slight pressure. The  $\text{SO}_2$  gas attacks certain of the non-sulfid minerals and products and combines with them, forming water 70 soluble sulfites, which are dissolved in the water contained in the pulp; the sulfites are then rapidly oxidized into sulfates by the oxygen of the hot air. Since the pulp enters one end of the drum cold and the  $\text{SO}_2$ - 75 charged air enters the opposite end hot, a counter current flow is developed which heats the water contained in the pulp say to a temperature around 40° C. near the discharge end of the drum. Since hot solutions 80 expel  $\text{SO}_2$  readily, this gas is forced forward toward the colder section of the drum and there is a constant counter current flow of  $\text{SO}_2$  gas toward the entering cold pulp. The internal construction of the drum insures 85 an intimate contact of the gas and mineral particles. The discharge is a practically neutral solution containing in the form of sulfates all the original  $\text{SO}_2$  soluble contents 90 of the charge. The particular element or elements sought may be recovered from these 95 solutions by whatever process is applicable.

100 As an example of the operation of this apparatus I will describe its application to extraction of copper from oxidized or non-sulfid ores thereof.

105 Ore pulp consisting of finely divided ore and water is fed in at opening 5 and the oxidized or non-sulfid constituents of the ore, consisting of carbonates, silicates, oxid 110 and metal, are subjected to the attack of the  $\text{SO}_2$  which is at this point practically exhausted. This is the first stage of the leaching. In the central part of the drum the copper is almost completely brought into 115 solution as sulfite. By the time it reaches this point, the gas is cooled by contact with the pulp,  $\text{SO}_2$  is thoroughly absorbed, and the reactions involving the solution of the copper minerals are practically complete. 120

At the outflow end of the drum the pulp is in contact with hot gas coming direct from the furnace and toward this end of the drum the oxidation of sulfites to sulfates is brought about. The absorption of  $\text{SO}_2$  in the hot pulp at this point is very small. The result is a counter current with respect to copper minerals and  $\text{SO}_2$ . Fresh ore is in contact with a practically exhausted gas. The exhausted ore is in contact with a gas high in sulfur dioxid. Toward the discharge end the oxidation of copper sulfite to sulfate is completed, and the high temperature insures that very little  $\text{SO}_2$  will remain in the pulp at this point.

The effect of the extracting and oxidizing operation above set forth is to bring the copper into solution in the form of copper sulfate, which is readily available for the recovery of the copper by any well known means. For example, the copper may be recovered by electrolysis of the copper sulfate solution, or by precipitation with iron, as cement copper. In each of these cases, the copper solution may be separated from the gangue or residue by filtration or otherwise before separation of the copper. If desired, however, the copper may be recovered by precipitation of metallic copper in the body of ore pulp, for example, by metallic iron agitated with the pulp, including the pregnant solution, and the whole body of pulp including the gangue and the precipitated copper and any undissolved copper values may then be subjected to flotation to separate the precipitated metallic copper together with any sulfid copper mineral that may be present.

In applying the above described apparatus to the recovery or concentration of manganese from its ores, a manganese ore, containing, for example, pyrolusite, may be made into pulp with water by suitable means, and supplied through chute 3 to drum 1 and passed through the same in contact with the sulfurous gases and air in the manner above described, with the result that the manganese is brought into solution in the form of manganese sulfate. Iron and lime are the main sulfurous acid soluble impurities usually associated with manganese ores and in the above described operation the lime oxidizes to sulfates and passes out with the non-solubles. The iron may be eliminated from the solution by reusing the solution on a new manganese charge, the manganese oxidizing the iron

and replacing it in solution and the iron being precipitated, probably as a basic salt. The solution of manganese sulfate, which is 60 eventually obtained may be treated by evaporation or crystallization to obtain the sulfate in solid form and this may be treated in any suitable manner for recovery of the manganese in commercially available form, 65 for example, carbon may be mixed with the sulfate and the mixture then roasted so as to produce oxid of manganese which is available as a commercial product. At the same time,  $\text{SO}_2$  gas is expelled and may be 70 used in carrying out the process above described for treatment of a fresh quantity of ore.

What I claim is:—

1. An apparatus for extracting metals 75 from their ores and oxidizing the resulting solution, consisting of a rotary drum provided with means for supply of ore pulp and outflow of gas at one end, and with means for outflow of ore pulp at the other 80 end, means for supplying hot sulfurous oxidizing gases to the drum at the pulp discharge end thereof, so as to cause such gases to pass through the drum in counter current with the ore pulp, said drum being 85 provided with lifts for raising the ore pulp and dropping it through the gases passing in the drum and with baffle means extending within the drum in position to intercept and distribute the ore pulp dropping from said 90 lifts.

2. An apparatus for extracting metals from their ores, comprising a rotary drum, provided at one end with a pulp inlet and gas outlet, and at the other end with a pulp 95 outlet and gas inlet, whereby ore pulp and gas may be passed in counter current through the drum, said drum having a series of perforated partitions extending across the drum, a series of bucket lifts extending adjacent to the peripheral wall of the drum and adapted to lift the ore pulp and drop it through the gas passing in the drum, and baffle bars extending longitudinally in the drum in position to intercept the ore pulp 100 105 descending from the lifts.

3. An apparatus according to claim 2 wherein said baffle bars are arranged in staggered relation in a plurality of annular series.

In testimony whereof I have hereunto subscribed my name this 15th day of June 1918.

EDMUND S. LEAVER.